

Patented Oct. 13, 1925.

1,557,367

# UNITED STATES PATENT OFFICE.

HERMANN KÄNDLER, OF BERLIN-FRIEDENAU, GERMANY, ASSIGNOR TO SIEMENS-SCHUCKERTWERKE GESELLSCHAFT MIT BESCHRÄNKTER HAFTUNG, OF SIEMENS-STADT, NEAR BERLIN, GERMANY, A CORPORATION OF GERMANY.

## PROCESS FOR INCREASING THE STRENGTH OF METALLIC BODIES.

No Drawing.

Application filed December 20, 1923. Serial No. 681,849.

*To all whom it may concern:*

Be it known that I, HERMANN KÄNDLER, a citizen of the German Empire, residing at Berlin-Friedenau, Germany, have invented 5 certain new and useful Improvements in a Process for Increasing the Strength of Metallic Bodies, of which the following is a specification.

This invention relates to a process for 10 treating or preparing metallic bodies for resistance tests or for increasing their strength.

For many purposes in the engineering industry and in particular for the construction 15 of motors, it is not sufficient to know the strength of the materials, such as iron and steel under tension, compression, bending stresses and the like, but it is also necessary to know their resistance to continuously 20 changing stresses. In particular the results of continuous shock, blow or impact tests (continuous shock bending tests) have attained particular importance in the arts. These tests permit, however, in comparison 25 with the tensile strength tests not sufficiently certain conclusions, parallel tests with similar test bodies of the same material frequently showing widely deviating fracture values. It was therefore hitherto necessary 30 to carry out a large number of parallel tests to obtain a fairly reliable result.

The present process is based upon the observation that the cause for the considerable 35 differences in the results of the tests is to be found in the fine cracks, fissures or scratches, which form on the surface of the test pieces during their preparation, particularly in the bottom of the notches made in such test pieces. Such fissures invariably 40 form the starting point of the fracture, although they may be only the very finest scratches produced during polishing. According to the size and shape of these fissures, which may hardly be perceivable by 45 the naked eye, sooner or later a permanent fracture is developed owing to the so-called notch action, the material at the surface being again and again strained beyond the elastic limit in consequence of the local 50 crowding of stresses.

These drawbacks are considerably lessened if not entirely eliminated according to this invention by attacking the surface of the test body or at least of the notch bottom by

physical or chemical means, which are capable of removing all discontinuities in the surface structure, by seizing or attacking smaller particles than mechanical means, such as the highest grade tools, are capable of doing. If such means are employed the sharp fissures disappear and a dull but uniform and continuous surface is produced. 55

Such means are for instance emanations in which the particles may be ejected from the surface of the body itself (cathode atomization) or in which the surface may be bombarded by foreign particles (cathode rays). 65

Chemical means may also be employed, for instance corroding agents, which dissolve the surface with which they are brought in contact. Heating up to the fusing point of the material also attains the end in view. The effect of the heat must, however, be confined to the most extreme outer layer, so that the structure of the 75 lower layers is not changed or injured.

By employing all these various means a particularly favorable circumstance aids the carrying out of the invention, viz, the fact, that all the forces which are capable to 80 engage the small particles of the surface at all operate automatically towards a removal of the unevennesses in the surface. In regard to the cathode rays this fact does not appear to call for a special explanation. 85 All projecting portions are to a higher degree exposed to the impact of the bombarding particles and are quickly levelled by them, while recesses, cracks and the like remain at first protected against the effect 90 of the bombardment.

In the chemical action by dissolving or corroding agents the same effect is attained. It is a well known fact, that a corroding agent attacks prominent portions far more 95 readily and removes them more speedily than cavities, which are generally only broadened at the bottom. This also occurs under the minute conditions with which we are concerned here. A scratch or fissure in the surface first offers its edges or burrs to the corroding agent and only gradually the action of the agent extends to the walls situated further in the interior and the bottom of the cavity is hardly attacked at all. 100 The crack or fissure thus gradually disappears and its place is taken by a smooth concave recess or flute which has less of a 105

notch or wedge action than the sharp fissure which it has displaced.

Test bodies of steel or other chemically composed substances are preferably treated 5 not with one corroding liquid only, but with a number of different ones. These need not be mixed together, but may be employed alternately or successively. The additional corrosive agents are intended to dissolve the 10 constituents which have not been sufficiently dissolved by the preceding agent.

The body to be treated may also be made 15 the cathode of a vacuum tube. The cathode rays emanating from it then first level all projecting parts, such as the edges of cavities and cracks or scratches, so that here also dangerous discontinuities in the surface and sudden changes in the cross-section of the body are avoided.

20 The fact that by fusing the most extreme outer surface layer by the application of temperatures up to the fusing point all sharp projections collapse and flow into the recesses or cavities can also be utilized 25 for carrying out this invention.

The drawbacks mentioned in connection 30 with the continuous shock bending tests, which result from the traces left by the treatment of the surface of the construction elements appear in conjunction with all kinds of stresses which are liable to lead to permanent fractures, in particular in the case of oscillation stresses of all kinds. Thus in all tests aiming at the 35 termination of the permanent strength the possibility is given to eliminate the discrepancies which otherwise exist in the results of parallel tests.

It is not claimed as new to remove coarse 40 cracks or fissures, which have obviously increased owing to continuous strains and have been recognized as starting points of an incipient permanent destruction, by milling or otherwise mechanically cutting the 45 material away, so that a hollow or concave flute or recess-bead or channel is formed.

The invention is based upon the recognition, that not only such cracks which may be traced easily by the naked eye become 50 gradually enlarged and finally cause a permanent fracture, but that discontinuities even of microscopic minuteness form the starting point for permanent fractures. As

no mechanical tool is capable of producing a surface, which is free from such fine irregularities or flaws, physical or chemical agents are according to this invention utilized, which are capable of dealing with such minute particles of the surface structure which are beyond the reach of mechanical tools. The means employed according to this invention operate essentially in the same manner in conjunction with very fine cracks or fissures as the mechanical tool in conjunction with coarse cracks 60 or rents.

The process is particularly useful for producing test pieces of materials, but may also be employed for treating parts of machines or building constructions before assembly or erection with a view of increasing their strength. Parts of their surface which appear particularly endangered may also after their assembly be treated in the manner described.

Frequently it will be advisable to carry 75 out the treatment after the machines or structures have been in service for some time and cracks or the like have appeared on the surface, in order to eliminate the 80 danger that such cracks become the source or starting point of the permanent destruction.

What I claim as my invention and desire to secure by Letters Patent is:—

1. A process of increasing the strength of a metallic body, which consists in removing discontinuities in its surface by means, capable of attacking smaller particles of the surface structure than can be removed by 85 mechanical means.

2. A process of increasing the strength of a metallic body, which consists in removing discontinuities in its surface by chemical means capable of attacking 95 smaller particles of the surface structure than can be removed by mechanical means.

3. A process of increasing the strength of a metallic body, which consists in subjecting the surface of the body successively to 100 the action of different corroding agents to remove discontinuities in the body surface beyond the reach of mechanical tools.

In testimony whereof I affix my signature.

HERMANN KÄNDLER.